

1

2,795,596

## FLEXIBLE WAX AND METHOD FOR PRODUCING SAME

Helmut Kolling, Duisburg-Hamborn, and Friedrich Rappen, Oberhausen-Sterkrade, Germany, assignors to Ruhrochemie Aktiengesellschaft, Oberhausen-Holten, Germany, a corporation of Germany

No Drawing. Application May 20, 1954,  
Serial No. 431,279

Claims priority, application Germany May 23, 1953

9 Claims. (Cl. 260—450)

This invention relates to flexible wax.

It is possible by means of catalytic carbon monoxide hydrogenation to produce paraffin waxes having very large molecular sizes which in contrast to normal slab paraffin derived from petroleum exhibit considerably higher melting points and a substantially higher hardness. These properties are very desirable in the production of wax impregnated paper. Unfortunately, however, these so-called hard paraffins gained from catalytic carbon monoxide hydrogenation are extremely brittle so that their use for paper impregnation is very limited.

The flexibility of waxes may be determined in the following manner:

A black paper strip is coated on both sides with a film of the paraffin to be tested of 0.01 mm. in thickness. This corresponds to a quantity of about 15–20 grams of paraffin per square meter of paper which is the amount most commonly applied in commercial practice. The application of the coating to the paper is effected in the laboratory by a process similar to that used in commercial manufacture. The coated paper strip is then stretched from both sides over a rotatable mandrel of about 4 mm. in diameter and the ends are pulled several times vertically up and down past each other. Depending upon the brittleness of the paraffin used, the wax film on the paper will rupture more or less. The measurement of the degree of rupture is effected photometrically by determining the brightening developed by the rupture of the film. This value is best determined by means of a photometer by means of which the percentage of the incident light reflected is measured. With normal slab paraffin, for example, a whiteness of 4 is measured which means that only 4% of the incident light is reflected while 96% is absorbed. Using hard paraffins obtained by catalytic carbon monoxide hydrogenation, a value of about 20 is obtained since the film produced from the hard paraffin becomes nearly completely ruptured during the treatment described above.

When, in paper impregnation, coatings are to be obtained which are harder and more temperature-resistant than those obtainable with pure normal slab paraffin, the so-called microcrystalline waxes must generally be used. Waxes of this type may be recovered from certain petroleum fractions by relatively costly processing methods. They have pour points of 70 to 90° C. and penetration numbers of generally between 3 and 20 at 20° C. The corresponding values of normal slab paraffin, as is known, range between 50 and 55° C. and 10 to 20 respectively. When measuring the flexibility in the manner described above, values of between 4 and 10 are obtained depending on the type of wax tested.

Owing to their higher melting points, these microcrystalline waxes are more temperature-resistant than normal slab paraffin. This temperature-resistance may be determined by a simple method. A paper strip is used which is coated with the particular wax. In order

2

to simulate actual service conditions, it is expedient to use the wax film which has previously been subjected to the flexibility test. If water of rising temperature is allowed to act from one side upon the paper strip which has been coated on both sides with wax, it can be observed that water drops will commence to pass through the paper at a certain temperature. This point will hereinafter be referred to as temperature-resistance. The temperature-resistance of microcrystalline waxes ranges between about 60° and 85° C. depending on the type of wax while with normal slab paraffin, water will pass through at a temperature of as low as 50° C.

Microcrystalline waxes are used in many cases in the production of floor and boot polishes to improve the retention properties of the pastes, i. e. the ability to retain solvents without loss. They are extensively used at the present time as a substitute of the naturally occurring ozocerite. Hard paraffin from catalytic carbon monoxide hydrogenation does not exhibit these retention-improving properties to a sufficient degree.

One object of this invention is the production from hard paraffin derived from catalytic carbon monoxide hydrogenation of a wax having properties of flexibility, temperature-resistance and retention-improving properties at least corresponding to those of microcrystalline waxes. This and still further objects will become apparent from the following description:

It has now been found that flexible and temperature-resistant waxes having retention-improving properties corresponding to the different types of microcrystalline waxes on the market may be produced from hard paraffin derived from catalytic carbon monoxide hydrogenation, if more than 1 and less than 6 gram atoms of chlorine, and preferably between 2 and 4 gram atoms of chlorine, are added to one mol of hard paraffin and the reaction product is subsequently subjected to a dehydrochlorination.

Hard paraffins melting between 90° and 120° C. may be produced in the conventional manner by means of the catalytic carbon monoxide hydrogenation with the use of cobalt or iron catalysts which are known per se. The method of producing hard waxes of this kind and the properties thereof have frequently been described in the literature.

It is known to chlorinate saturated hydrocarbons and to subsequently split off hydrogen chloride from the chlorination products in order to obtain hydrocarbons of the same structure having olefinic double bonds. This working method, however, involves in most cases the addition of far less than 1 gram atom of chlorine, as, for example, 0.5 gram atoms of chlorine per mol of hydrocarbon in order to obtain as high as possible a portion of mono-olefinic products. Hard paraffin, when subjected to this treatment, yields an olefinic product, the flexibility of which is practically the same as that of the starting material. Also, the molecular weight of the product has only minimally changed. It increases, for example, from 650 (starting material) to 680. In accordance with the invention, however, when more than 1 gram atom and less than 6 gram atoms of chlorine, and preferably 2 to 4 gram atoms of chlorine are added to each mol of hydrocarbon, there result flexible waxes which absolutely correspond to the microcrystalline petroleum waxes and have none of the brittle properties of the hard paraffin. The molecular weights of products of this type range between 800 and 1000.

It is advantageous to hydrogenate the reaction products after the dehydrochlorination. In this manner, a substantial brightening of the color is obtained. Moreover, the waxes lose their tackiness without detracting from their flexibility. It is the combination of chlorination and

dehydrochlorination with a hydrogenation which constitutes the fundamental difference between the process of the invention and the known production of olefinic hydrocarbons by chlorination and dehydrochlorination, the finished products of the process of the invention no longer having any olefinic double bonds.

The chlorination is effected in the known manner by introducing chlorine into the molten hard paraffin at temperatures ranging 10-20° C. in excess of the melting point of the hard paraffin being processed. The working conditions usually employed in the chlorination of hydrocarbons are known to anyone skilled in the art thus eliminating the necessity of giving particulars as to this step. The dehydrochlorination is effected by heating the chlorinated product for several hours at temperatures of between 280 and 320° C. and preferably of 300° C. and at normal atmospheric pressure or an elevated pressure of as high as 2 kg./square centimeter. It is also possible to effect the dehydrochlorination of reduced pressures, as, for example, at an absolute pressure of 0.5 kg./square centimeter. It is of advantage during the dehydrochlorination to add small amounts of activated carbon. The hydrogenation is preferably effected at temperatures of 200-280° C. and pressures of 100-200 kg./square centimeter with the use of hydrogenation catalysts which are known per se, as, for example, nickel or cobalt catalysts. The hydrogenation may be effected batchwise by the slurry process or continuously with fixed bed catalysts. The hydrogenation period amounts to about 1-3 hours.

It is of advantage in some cases, if relatively small amounts of low pour point portions which generally amount to 5-15% of the total product are separated by extraction from the reaction product after the dehydrochlorination and hydrogenation. This extraction is effected by treating the reaction product with 2 to 5 times its quantity of solvent at temperatures of 20-40° C. Suitable solvents are preferably hydrocarbons as, for example, hexane or heptane, chlorinated hydrocarbons, as, for example, dichloroethane, oxygenated hydrocarbons, as, for example, methanol and acetone, or mixtures of different solvents. It is of advantage to disperse the paraffin by spraying prior to the extraction.

A hard paraffin obtained by catalytic carbon monoxide hydrogenation, i. e. hydrocarbons boiling above approximately 400 or 450° C., is expediently used as the starting material for the process of the invention. Certain fractions of hard paraffin which may be recovered therefrom by distillation, crystallization or extraction processes are also suitable as starting material for the process of the invention. It is possible in this manner to prepare high melting point flexible waxes having specific properties.

The microcrystalline petroleum waxes include products with setting points of 65-70° C. which have a flexibility of 4. The flexibility of these waxes, however, is actually better than that of the normal slab paraffin or that of the microcrystalline waxes with pour points of about 75° C. It is also better than the flexibility of the waxes prepared in the manner described above, although the flexibility in all these cases is about 4.

For the determination of the higher flexibility, strips of about 0.5 mm. in thickness, 50 mm. in length of 15 mm. in width are cut out from the wax to be tested. These strips are stretched over a round stick of about 1 mm. diameter so that the ends of the strip extend vertically downward. A wax strip from the above described petroleum waxes with setting points of 65-70° C. will not break when being subjected to this severe test while strips of other waxes, when subjected to this treatment, will break to a more or less large extent although they have also a flexibility of 4.

It is also possible by the process of the invention, to obtain waxes which meet the severe flexibility test mentioned above in spite of having a much higher setting point as compared with commercial microcrystalline waxes, if the reaction period of the dehydrochlorination is extended to

more than 10 hours and preferably to 20 to 40 hours. With the dehydrochlorination effected within 3 to 5 hours, the olefinic product contains residual contents of chlorine of 0.1 to 0.3% which are still somewhat reduced in the subsequent hydrogenation. It is not possible by an extended dehydrochlorination period to achieve a substantial decrease of the residual content of chlorine. The extension of the dehydrochlorination period has, however, the surprising advantage that the quality of the reaction products undergoes a substantial improvement.

This mode of operation results in waxes which meet the aforesaid severe flexibility test just as well as microcrystalline petroleum waxes having a setting point of 65° to 70° C. In contrast to petroleum waxes, however, these waxes have setting points of 80 to 85° C. Thus, it is not only possible in accordance with the invention to fully reach the extremely good flexibility of some microcrystalline petroleum waxes but also to achieve in addition a substantial increase in the setting point. In this manner, there are obtained products which are far superior to all flexible waxes hitherto on the market.

The improvement of the quality of these waxes becomes particularly apparent if the waxes are separated into individual fractions by extraction with solvents as, for example, with heptane or dichloroethane. For this purpose, the extraction is carried out at increasing temperatures in such a manner as to extract at first 20% by weight of the material, then again 20% by weight thereof from the remaining extraction residue and so on, until the last fraction remains which, in the following table, is designated with "80 to 100% by weight."

The extraction was applied in the same manner to a wax obtained in accordance with the invention with the use of both, a short and a long dehydrochlorination period. As is to be noted from the flexibility values given in the table, all of the individual fractions of the wax according to the invention exhibit low flexibility values. However, the last extract fractions of the wax prepared with a short dehydrochlorination period show considerably poorer flexibilities. The presence of fractions of poor flexibility in the waxes prepared with a short dehydrochlorination period cannot be ascertained in determining the flexibility of the total wax. The poor flexibility, however, of the last extract fractions may be the reason why the wax prepared with a short dehydrochlorination period does not meet the severe flexibility test while the wax prepared with a long dehydrochlorination period entirely meets these conditions.

| 50   | Extract fraction, percent by weight | Whiteness                 |                          |
|------|-------------------------------------|---------------------------|--------------------------|
|      |                                     | rapid dehydrochlorination | slow dehydrochlorination |
| 55 I | 0-20                                | 4.0                       | 4.0                      |
| II   | 20-40                               | 4.3                       | 4.1                      |
| III  | 40-60                               | 4.8                       | 4.3                      |
| IV   | 60-80                               | 6.1                       | 4.4                      |
| V    | 80-100                              | 8.6                       | 4.6                      |

60 The waxes prepared in accordance with the invention have properties which correspond in every respect to those of the microcrystalline waxes on the market. The waxes may be used with particular advantage for paper impregnation. They may also be used, however, as a substitute of ozocerite because they have an extremely good retention effect, that is to say, even small portions effect a very considerable reduction of the solvent loss of pastes.

65 The process of the invention has the advantage that waxes which are equivalent in every respect to the so-called microcrystalline waxes obtained from petroleum may now be prepared from synthetic hydrocarbons. Moreover, the properties of these waxes may be varied within wide limits depending upon the reaction conditions chosen. Starting 70 with the hard paraffins derived from catalytic carbon

monoxide hydrogenation which are readily available in large amounts, the process of the invention allows the production of any wax type desired in any quantity and in a relatively simple and cheap manner.

*Example 1*

Hard paraffin derived from catalytic carbon monoxide hydrogenation and containing only hydrocarbons boiling above 460° C., having a setting point of 100° C. and a penetration number at 20° C. of 0.5 was chlorinated at 110-120° C. with irradiation and stirring until 1.5 gram atoms of chlorine had been absorbed per mol of hydrocarbon. The chlorinated product was mixed with 1% activated carbon and heated for 3 hours at 300° C. while stirring and passing through small amounts of nitrogen. After having filtered off the active carbon, a weakly yellowish reaction product was obtained which had a setting point of 89° C. and a penetration number of 7.5. The determination of the flexibility effected in the manner described in the description of the invention resulted in a number 5. The temperature-resistance was 75° C. The hard paraffin used as the starting product showed a value of 20 when subjected to the flexibility test.

*Example 2*

The finished product of Example 1 was stirred for 30 minutes at about 20° C. with two times its quantity of ethylene chloride and subsequently filtered. In addition to 10% of extract there was obtained a weakly yellowish extraction residue which had a setting point of 91° C., a penetration number of 3, a whiteness of 6 as determined by the flexibility test, and a temperature resistance of 80° C.

*Example 3*

Hard paraffin of the type used in Example 1 was chlorinated until 2 gram atoms of chlorine per mol of hydrocarbon had been absorbed. After the dehydrochlorination which in this experiment was effected for 4 hours at about 300° C., there resulted a weakly yellowish product which had a setting point of 85° C., a penetration number of 17, a value of 4 as determined by the flexibility test, and a temperature resistance of 70° C.

*Example 4*

Hard paraffin of the type used in Example 1 was chlorinated until 2.5 gram atoms of chlorine per mol of hydrocarbon had been absorbed. After the dehydrochlorination which was effected in the manner set forth in Example 3, there resulted a yellowish product which had a setting point of 82° C., a penetration number of 34, a value of 4 as determined by the flexibility test, and a temperature resistance of 65° C.

*Example 5*

Hard paraffin of the type used in Example 1 was chlorinated until 3 gram atoms of chlorine per mol of hydrocarbon had been absorbed. After the dehydrochlorination which was effected for 5 hours at about 300° C., the reaction product was hydrogenated with hydrogen using a nickel catalyst. After having filtered off the catalyst, there resulted a white reaction product which was subsequently stirred for 30 minutes at about 20° C. with two times its quantity of ethylene chloride. In addition to 14% extract, there was obtained a product which had a setting point of 91° C., a penetration number of 3.5, a value of 7 as determined by the flexibility test, and a temperature resistance of 82° C.

*Example 6*

Hard paraffin of the type used in Example 1 was chlorinated until 4 gram atoms of chlorine per mol of hydrocarbon had been absorbed. After the dehydrochlorination and subsequent hydrogenation, effected in the manner set forth in Example 5, there was obtained a white reaction product which had a setting point of 85° C., a

penetration number of 22, a value of 4 as determined by the flexibility test, and a temperature resistance of 65° C.

*Example 7*

5 A paste was prepared from 6 parts by weight of the hard paraffin used in Example 1, 24 parts by weight of slab paraffin having a setting point of 50-52° C., and 70 parts by weight of a mixture of solvent naphtha and turpentine. This paste was placed in an air conditioning box for free evaporation at 20° C. The retention number measured after 10 days was 30.

10 The retention number of a paste consisting of 4.8 parts by weight of the hard paraffin used for Example 1, 1.2 parts by weight of commercial ozocerite having a setting point of 70° C., 24 parts by weight of slab paraffin and 70 parts by weight of a mixture of solvent naphtha and turpentine amounted to 20 after 10 days.

15 If the commercial ozocerite in the paste was replaced by the finished product of Example 1, then this paste had a retention number of 12 after 10 days.

*Example 8*

20 Hard paraffin derived from catalytic carbon monoxide hydrogenation, containing only hydrocarbons boiling above about 450° C., having a setting point of 96° C. and a penetration number of 1.0 was chlorinated at 110-120° C. with irradiation and stirring until 3.5 gram atoms of chlorine had been absorbed per mol of hydrocarbon. The chlorinated product was mixed with 1% active carbon and heated for 40 hours at 300° C. while stirring and passing through small amounts of nitrogen. After having filtered off the solid constituents, there resulted a yellowish reaction product which contained 0.1% chlorine.

25 The olefinic hydrocarbon mixture was hydrogenated in a pressure vessel provided with a stirrer with hydrogen for 3 hours at 200-250° C. and a pressure of 120-150 kg./square centimeter using a nickel catalyst. After having filtered off the catalyst, there resulted a weakly yellowish product which had a setting point of 83° C.

30 A strip of 0.5 mm. in thickness, 50 mm. in length and 15 mm. in width was cut out from the wax thus prepared. This strip of wax was bent over a round stick of 1 mm. diameter so that the two ends of the strip extended vertically downward. No rupture of the wax strip could be observed.

35 The process in accordance with the invention permits the production of any type of commercial waxes having microcrystalline structures by varying the quantity added of chlorine within the interval in accordance with the invention of 1-6 gram atoms of chlorine per molecule of hydrocarbon, by varying the temperature and duration of the dehydrochlorination and the conditions of the hydrogenation. The above examples serve only to illustrate the process of the invention. Anyone skilled in the art will be able to derive therefrom working conditions according to the invention for the production of similar flexible waxes.

40 We claim:

45 1. Process for the production of flexible waxes from hard paraffins derived from catalytic carbon monoxide hydrogenation which comprises chlorinating such a hard paraffin with more than 1 and less than 6 gram atoms of chlorine per mol, heating the chlorinated product at a temperature of 280 to 320° C. to effect a dehydrochlorination of said product and recovering the flexible wax formed.

50 2. Process according to claim 1 in which said chlorination is effected with 2 to 4 gram atoms of chlorine per mol of paraffin.

55 3. Process according to claim 1 which includes catalytically hydrogenating the reaction product after said dehydrochlorination.

60 4. Process according to claim 1 which includes extract-

70 75

ing the low pour point portions from the recovered flexible wax.

5. Process according to claim 1 in which the chlorinated product is heated at a temperature of 280 to 320° C. for at least ten hours for said dehydrochlorination.

6. Process according to claim 5 in which said chlorinated product is heated at a temperature of 280 to 320° C. for 20 to 40 hours for said dehydrochlorination.

7. Process according to claim 1 in which said dehydrochlorination is effected at a temperature of about 10 300° C.

8. A flexible wax produced by chlorinating with more than one and less than six gram atoms of chlorine per mol, a hard paraffin fraction, derived from catalytic carbon monoxide hydrogenation, consisting of hydrocarbons boiling above 400° C. and thereafter dehydrochlorinating the chlorinated product by heating to a temperature of 280° to 320° C.

9. A flexible wax produced by chlorinating with more

than one and less than six gram atoms of chlorine per mole, a hard paraffin fraction, derived from catalytic carbon monoxide hydrogenation, consisting of hydrocarbons boiling above 400° C., dehydrochlorinating the chlorinated product by heating to a temperature of 280° to 320° C., and thereafter catalytically hydrogenating the dehydrochlorinated product.

References Cited in the file of this patent

UNITED STATES PATENTS

|           |                |               |
|-----------|----------------|---------------|
| 2,587,588 | Berry          | Mar. 4, 1952  |
| 2,597,908 | Stewart et al. | May 27, 1952  |
| 2,597,910 | Thaw et al.    | May 27, 1952  |
| 2,651,655 | Loughran       | Sept. 8, 1953 |
| 2,658,090 | Geiser et al.  | Nov. 3, 1953  |

FOREIGN PATENTS

|         |               |              |
|---------|---------------|--------------|
| 505,898 | Great Britain | May 12, 1939 |
|---------|---------------|--------------|